

## UNITED STATES PATENT OFFICE

2,516,536

## PURIFICATION OF BRASSES AND BRONZES

William F. Tschappat, Pittsburgh, Pa., assignor  
to The American Metal Company, Limited, New  
York, N. Y., a corporation of New York

No Drawing. Application January 22, 1948,  
Serial No. 3,830

3 Claims. (Cl. 75—76)

1

This invention relates to the purification of brasses and bronzes and particularly to the removal of sulfur from such metals in an economical manner to produce such metals with a lowered sulfur content.

The patent to Hanak 1,837,432, patented December 22, 1931, is known to me. It employs a mixture of metallic sodium and sodium carbonate for purification of copper alloys such as brass. So far as I am aware, this process has never been practiced. It is an expensive process because of the use of an expensive metal, viz., sodium or other alkali metal, which is an essential constituent of the bath according to Hanak. It has also been heretofore proposed, in accordance with another process, to use soda ash with coal or charcoal which is added to molten brass and rabbled into the mass. This method of combining the soda ash and brass has been found to have three major difficulties: (1) It takes a long time to remove the sulfur; (2) one treatment with soda ash and reducing agent under this old method usually results in relatively small elimination of sulfur and the method had to be repeated a number of times, and (3) due to the length of time necessary for the soda to be in contact with the brass, the wear-and-tear on the furnace linings is greatly increased. The process not only consumes considerable time with consequent wear-and-tear on the furnace linings, but it requires over twice as much labor. For instance, for handling the same amounts of brass or bronze as given in the examples below, five men were required in the operations of the old process for about 6 to 8 hours, while in accordance with my process, only two men were required for approximately two hours. Also, soda ash alone or with a reducing agent has been used by blowing it under the surface of the molten bath, but with about the same disadvantages as just mentioned.

The principal object of the present invention accordingly is to provide a process for purifying brasses or bronzes which will overcome at least some of the disadvantages of the prior processes and which will result in the economical removal of sulfur therefrom.

The invention accordingly comprises the novel processes and steps of processes, specific embodiments of which are described hereinafter by way

2

of example and in accordance with which I now prefer to practice the invention.

I have found that the reducing agent, namely, coal or charcoal, can be eliminated and the whole process can be greatly simplified and shortened and sulfur can be removed in one step during the melting-down period by first preparing a molten bath of sodium carbonate and then adding the brass to this bath in solid form. As the brass melts, it trickles through the sodium carbonate and removal of sulfur immediately occurs.

In carrying out my process, I charge from 5 to 15% of an alkali such as sodium carbonate or sodium hydroxide or other alkalies hereinbelow defined into an empty reverberatory furnace, for example. The percentage of such alkali charged is based on the weight of the brass or bronze to be treated. The sodium carbonate or other alkali forms a molten bath. While maintaining the bath above the melting point of the metal—brass or bronze—to be treated, the said metal is charged into the furnace as rapidly as possible and melted. The metal as it melts drips through the molten bath of alkali and produces a slag containing a large part of sulfur. The sulfur is apparently removed from the metal as a complex compound, mostly a mixture of sodium sulfide and sodium sulfite.

My method is especially useful in cleaning impure brasses or bronzes, especially those high in sulfur, such as cupola slabs, and serves to remove sulfur therefrom to produce either stock or finished ingots. By "stock ingots" is meant ingots containing, say, from .05 to, say .15% sulfur. These are useful for blending with other substantially sulfur-free brasses or bronzes or similar metal to produce metals conforming with all standard specifications.

The following are specific examples of my process. It is to be understood that these examples are illustrative only and that the invention is not to be confined thereto except as indicated in the appended claims.

45 Examples

1. Three thousand pounds of sodium carbonate was charged into a reverberatory furnace and caused to form a liquid bath having a temperature of about 2200° F. A charge of 26,018 pounds 50 of impure red brass in rough cast slabs contain-

ing sulfur and other ingredients as shown in the analysis below were then charged into the furnace as rapidly as possible and allowed to melt completely. The metal dripped through the molten sodium carbonate. The slag was then removed from the molten bath. The bath was well stirred and, upon analysis, it was found that the sulfur by this single treatment had been reduced from .50% to .11%. An analysis of the metal before and after treatment is given below, as well as an analysis of the slag.

| Analysis before Treatment |       | After Treatment |       | Slag Analysis |       |
|---------------------------|-------|-----------------|-------|---------------|-------|
| Cu.....                   | 79.74 | Cu.....         | 82.92 | Cu.....       | 3.68  |
| Sn.....                   | 5.42  | Sn.....         | 5.28  | Sn.....       | .81   |
| Pb.....                   | 7.32  | Pb.....         | 8.15  | Pb.....       | .13   |
| Zn.....                   | 3.49  | Zn.....         | 1.71  | Fe.....       | 12.73 |
| Fe.....                   | 2.03  | Fe.....         | .28   | S.....        | 2.49  |
| Sb.....                   | .60   | Sb.....         | .60   |               |       |
| Ni.....                   | .76   | Ni.....         | .85   |               |       |
| S.....                    | .54   | S.....          | .11   |               |       |
| Total.....                | 99.90 | Total.....      | 99.90 |               |       |

2. A larger lot of materials was employed in carrying out this second example, the melt being made in a larger furnace with somewhat faster melting of the soda ash and metal slags resulting in a single treatment in the removal of a larger amount of sulfur from the metal treated. Sixty-six hundred pounds of sodium carbonate was charged and allowed to become liquid and maintained at a temperature about 400° F., above the melting point of impure red brass. 65,603 pounds of impure red brass containing sulfur and other ingredients as shown below in slab shapes was charged into the furnace as rapidly as possible and allowed to melt completely. The red brass, as before, trickled through the molten bath of sodium carbonate and the sulfur was removed. The slag was then removed from the molten bath. The bath was well stirred and, on analysis, it was shown that the sulfur in the original metal, amounting to .50%, had been reduced to .05% sulfur. The analysis of the metal before and after treatment, as well as the slag analysis, is given below:

| Analysis before Treatment |       | After Treatment |       | Slag Analysis |      |
|---------------------------|-------|-----------------|-------|---------------|------|
| Cu.....                   | 79.74 | Cu.....         | 82.53 | Cu.....       | 6.58 |
| Sn.....                   | 5.42  | Sn.....         | 5.39  | Sn.....       | .36  |
| Pb.....                   | 7.32  | Pb.....         | 8.43  | Pb.....       |      |
| Zn.....                   | 3.49  | Zn.....         | 1.88  | Fe.....       | 7.33 |
| Fe.....                   | 2.03  | Fe.....         | .10   | S.....        | 5.70 |
| Sb.....                   | .60   | Sb.....         | .66   |               |      |
| Ni.....                   | .76   | Ni.....         | .86   |               |      |
| S.....                    | .54   | S.....          | .05   |               |      |
| Total....                 | 99.90 | Total....       | 99.90 |               |      |

3. Seven thousand pounds of sodium carbonate was charged and allowed to become liquid and maintained at a temperature about 400° F., above the melting point of impure red brass. 70,431 pounds of impure red brass containing sulfur and other ingredients as shown below in slab shapes was charged into the furnace as rapidly as possible and allowed to melt completely. The red brass, as before, trickled through the molten bath of sodium carbonate and the sulfur was removed. The slag was then removed from the molten bath. The bath was well stirred and, on analysis, it was shown that the sulfur in the original metal, amounting to .79%, had been reduced to .15% sulfur. The analysis of the metal before and

after treatment, as well as the slag analysis, is given below:

| Analysis before Treatment |       | After Treatment |       | Slag Analysis |      |
|---------------------------|-------|-----------------|-------|---------------|------|
| Cu.....                   | 85.01 | Cu.....         | 88.12 | Cu.....       | 7.62 |
| Sn.....                   | 4.83  | Sn.....         | 4.54  | Sn.....       | .32  |
| Pb.....                   | 4.68  | Pb.....         | 4.83  | Pb.....       |      |
| Zn.....                   | 2.47  | Zn.....         | .78   | Fe.....       | 6.58 |
| Fe.....                   | .65   | Fe.....         | .04   | S.....        | 5.90 |
| Sb.....                   | .24   | Sb.....         | .32   |               |      |
| Ni.....                   | 1.25  | Ni.....         | 1.01  |               |      |
| S.....                    | .79   | S.....          | .15   |               |      |
| Total.....                | 99.92 | Total.....      | 99.92 |               |      |

15. In place of sodium carbonate in the above examples, there may be substituted caustic soda NaOH, potassium hydroxide or potassium carbonate. These materials operate in the same manner and in equivalent proportions to give the same result but they are more expensive than the preferred sodium carbonate and the latter is more easily handled in the furnace.

Instead of brass, a similar weight of bronze may be substituted in the above examples.

20. In the appended claims, where the term "alkali" is used, it is intended to designate sodium carbonate, sodium hydroxide, potassium carbonate or potassium hydroxide.

What I claim is:

30. 1. A process for removing sulfur from impure brass containing same which comprises, preparing a molten bath of sodium carbonate in the proportion of about 5 to 15% thereof based on the weight of the impure brass charged and while maintaining such bath above the melting point of the brass to be treated, charging such brass in unmelted condition thereinto and rapidly completely melting the brass, allowing the molten brass to trickle through the molten carbonate to produce a slag containing a large part of the sulfur.

35. 2. A process for removing sulphur from impure brass or bronze metal containing same, which comprises preparing a molten alkali bath in the proportion of 5 to 15% of the weight of the metal charge to be purified while maintaining such bath above the melting point of the impure metal to be treated, charging such metal in unmelted condition into said molten bath and rapidly completely melting the brass, and allowing the molten metal to trickle through the molten alkali to produce a slag containing a large part of the sulphur.

40. 3. A process for removing sulphur from impure brass or bronze metal containing same, which comprises preparing a molten alkali bath in the proportion of 5 to 15% of the weight of the metal charge to be purified while maintaining such bath above the melting point of the impure metal to be treated, charging such metal containing 45. .5% to .6% sulphur in unmelted condition into said molten bath and rapidly completely melting the brass, and allowing the molten metal to trickle through the molten alkali to produce a metal which contains about .1 sulphur or less.

45. 60. WILLIAM F. TSCHAPPAT.

#### REFERENCES CITED

The following references are of record in the file of this patent:

#### UNITED STATES PATENTS

| Number    | Name          | Date          |
|-----------|---------------|---------------|
| 1,921,180 | Evans         | Aug. 8, 1933  |
| 1,921,868 | Evans         | Aug. 8, 1933  |
| 1,955,726 | Archer et al. | Apr. 24, 1934 |